

March 25, 1924.

1,487,719

H. T. CHANDLER  
PROCESS OF MALLEABLEIZING IRON

Filed Nov. 14, 1921



Fig. 2



Fig. 2

Inventor  
Henry Thomas Chandler

By Whittmore Hubert Whittmore  
+ Belknap Attorneys

## UNITED STATES PATENT OFFICE.

HENRY T. CHANDLER, OF MARYSVILLE, MICHIGAN.

## PROCESS OF MALLEABLEIZING IRON.

Application filed November 14, 1921. Serial No. 514,844.

*To all whom it may concern:*

Be it known that I, HENRY THOMAS CHANDLER, a citizen of the United States of America, residing at Marysville, in the county of St. Clair and State of Michigan, have invented certain new and useful Improvements in Processes of Malleableizing Iron, of which the following is a specification, reference being had therein to the accompanying drawings.

Commercially, the manufacture of malleable iron is conducted in two steps. The first of these includes melting, molding, casting and other foundry operations incident to the production of suitable white iron castings. The second step consists in the conversion of these hard, brittle, un-machineable castings, by a suitable thermal treatment, into soft, malleable and commercially useful products.

This invention relates particularly to this second step in the manufacture of malleable iron, which is known as annealing or graphitization, and has for its object; first, reduction in the time required for the completion of the process; second, greater efficiency; third, reduction in the cost of the installation required for the process; fourth, economy in space; fifth, the obtaining of a high grade product.

The nature of this process, its objects and advantages will be best understood after an elementary description of the chemistry of graphitization and an outline of the usual commercial method of annealing.

Metallurgically, white iron, suitable for malleableizing, consists of a mixture of iron carbide, known as cementite, and an alloy of iron carbide and iron. The properties of these constituents and their distribution within the casting account for the brittleness and other physical characteristics of the metal. This system, in which the carbon all exists in chemical combination, is metastable; in other words, it is permanent not because actual chemical equilibrium exists, but because further molecular re-arrangement is impossible under the temperature conditions obtaining. It is the purpose of annealing to convert, by the effect of time and temperature, this metastable system of iron carbide and iron into the stable system consisting of iron and free carbon (graphite), accomplishing thereby a change in the nature and re-arrangement of the constitu-

ents of the casting resulting in a commercially useful product.

Annealing practice, as usually carried out, consists first in packing the castings together with either an inert or chemically active material, such as mill scale, slag, iron ore and the like, in cast iron or other pots. Various sizes and forms of containers and kinds of packing materials are used, depending largely upon the work to be treated and to some extent upon the nature of the equipment available and personal opinion of the annealer. The purpose of packing is primarily to support the castings while hot and thus prevent sagging or distortion under their own weight or the weight of the castings above them. It also serves as a protection for the castings from scaling or other effects of the combustion gases and further, due to mass, has a stabilizing effect upon temperature, preventing rapid changes harmful to this process. Packing has no significant effect upon the graphitizing reactions proper.

The pots containing the castings are then stacked and charged into the annealing ovens. These ovens are usually very simply constructed and hand fired with coal. They may hold from twenty-five to one hundred stacks of pots; neither extreme, however, is common practice. The doors are sealed and the oven and its contents are brought to a maximum temperature of from about 1500 to 1850 degrees Fahrenheit. The rate of heating is chemically unimportant and is limited by the nature of the oven and the disposition of the charge within.

Temperature is maintained for a period of from a few hours to several days, to effect thorough heating of the charge and permit the initial reactions within the castings to attain equilibrium. When this is accomplished, firing is stopped and the oven and contents allowed to cool. The cooling rate is important and the ovens are so built that this does not exceed 10 to 15 degrees per hour throughout the critical range. After cooling to from 1000 degrees Fahrenheit to around 200 degrees Fahrenheit, depending largely upon the means available for removing the work, the pots are removed and the castings cleaned, after which they are ready for use.

The complete annealing cycle as thus carried out requires from six days to, in some

cases, over two weeks. Wide variations in detail are practiced in different foundries, due, no doubt, to the fact that the art of producing malleable iron preceded by over a hundred years an understanding of the chemistry of graphitization.

In all instances, however, the complete process may be divided into the following four intervals, the first two of which being 10 heating and the last two cooling operations:

1st. Heating to some temperature above the  $A_1$  point.

2nd. Holding at this temperature for a period of time.

15 3rd. Cooling to below the  $A_1$  point at a slow rate.

4th. Further cooling to permit handling.

These four parts of the annealing cycle are completed in a single furnace or annealing chamber, substantially as outlined above.

20 The process, thus conducted, when compared with analogous metallurgical operations, is very inefficient. This is due; first, to the fact that an oven which will have the 25 slow cooling characteristics necessary for the successful completion of the process, is not a construction suitable for the efficient heating of the work either as regards time or fuel economy; second, the oven operates as 30 a heating unit during but a small part of the time necessary for the complete cycle; third, the extreme range of temperature to which the oven is subjected results in rapid deterioration and heavy upkeep expenses.

35 Initial installation, upkeep and overhead costs must, therefore, be met on an apparatus which is idle a greater part of the time in performing one of its major functions, which is subjected to temperature extremes,

40 causing rapid deterioration due to expansion and contraction of the brick work, and, due to the great length of time necessary to complete the process, is limited in its output. The direct result of these conditions 45 is that only the most simple and cheap constructions are economically practical, and more efficient furnaces and methods of fuel utilization, through almost universally used in allied practice, are here ruled out on the 50 basis of cost.

More recent development has contemplated the use of electricity as a source of heat or the use of muffle furnaces of either the stationary or tunnel type, in order to avoid 55 packing and thus speed up the process to a point where the use of such equipment becomes of economic value.

In the tunnel furnaces the work is gradually advanced, first passing through a zone 60 in which the proper temperature is reached and maintained and then through portions at progressively lower temperatures to completion. Such a type of apparatus is necessarily initially very expensive, due; first, to its large size; second, the muffle construction

necessary to avoid scaling; and third, to the mechanical equipment necessary to effect the movement of the charge through the furnace. Furnaces of this type can only be efficient when constantly operating at full 70 or nearly full capacity, and therefore lack the flexibility demanded in the usual jobbing foundry.

In the stationary type of muffle furnace, packing is also either totally or partially 75 eliminated, and the cooling cycle becomes a question of furnace control.

With my improved process, instead of carrying out the complete operation in one apparatus, the heating and cooling steps of the 80 treatment are separated and accomplished in different enclosures, the heating being carried on in a furnace which is adapted for efficiently carrying out this operation and the work being then transferred to an apparatus constructed to efficiently effect the necessary cooling cycle. The process is based; first, on the discovery that chemically 85 the rate of heating is immaterial; second, that the higher the initial temperature is 90 raised above the critical point, the more rapidly is chemical equilibrium established; third, that the rate of cooling is immaterial, excepting through a narrow temperature 95 range, and; fourth, that the initial temperature may be considerably higher than this range.

The conditions being such, the transfer of work to the cooling chamber may be accomplished without detriment to the reactions 100 of graphitization, it being only necessary that the initial temperature should be sufficiently high to avoid dropping below this critical range during transfer.

The specific form of apparatus required 105 for the carrying out of my improved process may be varied, but as diagrammatically represented in the drawings,

Figure 1 is a cross section through the 110 heating furnace; and

Figure 2 is a similar view through the cooling chamber.

As shown, A is a furnace suitably constructed for the efficient heating of the work placed in the chamber. The furnace may be 115 of the car type in which the work is placed upon trucks B which are movable into and out from the furnace, or any other convenient means of transportation may be provided. C is the cooling chamber which differs radically in its construction from A so as to be efficient in the control of the cooling of the work. If the work is placed on trucks, these may be transferred from the heating furnace A to the cooling chamber C 120 and these two parts of the apparatus may be located in any convenient relation to each other. Cooling may be controlled by the use of suitable dampers for the admission of hot waste gases from the melting furnaces 125

or heating oven, or the use of an individual heating equipment, or combinations of these. In place of cooling of the product of the heating chamber in a single cooling chamber, two or more of these may be used, if desired.

The essential feature of the apparatus is that the cooling chamber shall not interfere with the efficient functioning of the heating furnace and that the heating furnace shall not interfere with efficient functioning of the cooling chamber.

In operation, the higher the temperature in the heating furnace without detriment to the work, the more rapidly is equilibrium established in the initial reaction, and the shorter the time interval required for this step of the treatment. The work is therefore placed in the heating furnace and permitted to remain for an interval varying with the temperature and with other conditions, such as the analysis of the iron, the manner of packing, etc. The work is then transferred to the annealing furnace and the rate of cooling controlled until the low point of the critical range is reached, after which it may be removed.

The time required for the complete process as thus carried out is very much less than with the usual practice, as not only is heating effected more rapidly than in usual practice, but also the very slow cooling necessary to the reaction is carried out only within the range in which it is effective.

The economies of the process are many, among which may be cited the following:

First, the heating furnace is operated continuously as a heating unit within a comparatively narrow temperature range, thus varying fuel consumption;

Second, the cooling chambers are of very simple and cheap construction and are capable of long service, as they are not subjected to either excessive temperature or change of temperature;

Third, due to the resulting shorter time cycle, the output of the annealing equipment is increased and the overhead burden borne by the charge is reduced;

Fourth, installation costs are low when compared either with the usual practice or the use of tunnel and muffle furnaces.

What I claim as my invention is:

1. The method of malleableizing iron which consists in heating the work in one enclosure and in cooling the work in a separate enclosure.

2. The method of malleableizing iron which consists in heating the work in a furnace adapted for the efficient accomplish-

ment of such operation, in cooling the work in a separate chamber and in transferring the work from the one to the other while at a temperature above the critical point.

3. The method of malleableizing iron which consists in heating the work in a furnace adapted for efficient and rapid elevation of temperature to above the critical point for the primary reaction, in maintaining the temperature above such point until the equilibrium of the primary reaction is established, in transferring the work while at a temperature still above said critical range to a separate cooling chamber and in controlling the rate of cooling through the low point of the critical range.

4. The method of malleableizing iron which consists in elevating the temperature of the work rapidly to above the critical point (A<sub>1</sub>) for initiating the primary reaction, in a furnace adapted for efficiently accomplishing such treatment, in transferring the work while still above the critical temperature to a cooling chamber and in controlling the cooling process at the required rate through the critical range.

5. The method of malleableizing iron which consists in heating the work while stationary in one enclosure, in transferring the work to a separate enclosure, and cooling the work while stationary in the latter enclosure.

6. The method of malleableizing iron which consists in heating the work while stationary in a furnace adapted for the efficient accomplishment of such operation, in transferring the work while at a temperature above the critical point to a separate chamber adapted for controlling the rate of cooling and cooling the working in said chamber at a predetermined rate through the low point of the critical range while said work is stationary therein.

7. The method of malleableizing iron which consists in placing the work in a furnace adapted for efficient and rapid elevation of temperature to above the critical point for the primary reaction, in maintaining the work stationary in said furnace at a temperature above such point until the equilibrium of the primary reaction is established, in transferring the work while at a temperature still above said critical range to a separate cooling chamber, and in controlling the rate of cooling through the low point of the critical range while maintaining the work stationary in said chamber.

In testimony whereof I affix my signature.  
HENRY T. CHANDLER.